

## UNITED STATES PATENT OFFICE

1,999,316

## METHOD OF TANNING HIDES AND SKINS

Max Bergmann, Dresden, Germany, assignor to  
Studiengesellschaft der Deutschen Lederindus-  
trie G. m. b. H., Dresden, GermanyNo Drawing. Application May 7, 1932, Serial No.  
609,988. In Germany May 20, 1931

9 Claims. (Cl. 149—5)

It is universally known to use, certain chromic salts of synthetic tanning substances for tanning or dressing purposes which substances are formed by linking organic compounds and contain free 5 sulfo-groups.

Now, I have found that aromatic sulfonic acids having one nucleus or several nuclei and which in themselves possess no tanning properties and are not formed by linkage of organic molecules, can be utilized, in the form of chromic salts, for tanning purposes, especially for dressing hides or skins with the result of producing and obtaining leather of particularly valuable qualities.

Said chromic salts may be made in solid form adapted to be dissolved in a suitable liquid for the tanning purpose, but in many cases it may be preferable to use, in lieu thereof, solutions which have been made immediately from any appropriate organic or inorganic chromic salts and said aromatic sulfonic acids or sulfonates which in themselves are devoid of tanning faculties, said solutions thus containing chromic salts of sulfonic acids owing to a more or less extensive transposition.

In some cases I have found it advisable to have the said transposition or conversion of the chromic salts and the aromatic sulfonic acid or salt (sulfonate) take place immediately in situ, that is to say, within the hides or skins to be tanned, and in such a case I treat the hides or skins, in succession first with the one and subsequently with the other one of the two substances or components, whereupon I regulate the alkalinity to the required degree in the usual manner.

The employment of the described chromic salts for tanning purposes according to the present invention involves the advantage of considerably reducing the possibility or danger of producing leather of wrinkled or drawn grain as final product which is highly objectionable for known reasons, while on the other hand in most cases a well-grained, soft and full leather will be obtained, according to the present invention, without the necessity of subjecting the hides or skins to a preparatory treatment with any particular pickling agent or, as the case may be, any particular bating agent.

Furthermore, hides and skins treated in the manner herein described for tanning purposes and soaked after having been previously dried in the usual way, will rapidly absorb again the amount of water they have lost during the said drying operation, and they are just as well adapted to absorb fats and colouring matters with absolute uniformity.

The following examples will serve to illustrate the nature of the invention, but they are merely typical cases and can be varied without departure from the nature of the invention. The parts are by weight.

## Example 1

Properly prepared and pickled calf skins from which the hair has been taken off, are treated, for the tanning purpose, with a 2 to 3 per cent solution of p-toluol-sulfonate of chrome, the so-called hexaquio salt—see G. Jantsch and K. Mackenstock, Reports of the Vienna Academy of Science, 1929, Division II, vol. 138, pag. 337—, the said solution being controlled and adjusted to have a degree of alkalinity as required or suited for the tanning process as regards both the initial and the final condition thereof. The treatment of the skins may be carried out as described either in a vat or pit or on a reel or in any other suitable manner known in the art.

## Example 2

100 parts of calf skins properly bated but without having been previously subjected to a pickling treatment, are placed in a tanning liquor composed of 30 parts of chrome- $\beta$ -naphthalino-sulfonate and 750 parts of water and prepared to have an initial alkalinity or basicity of 20 percent and subsequently of 33 per cent.

The said chrome- $\beta$ -naphthalino-sulfonate may be made by dissolving 40 parts of chromic nitrate in 50 parts of water and mixing the resulting solution with a solution of 65 parts of  $\beta$ -naphthalino-sulfonic acid dissolved in 150 parts of water. Chrome- $\beta$ -naphthalino-sulfonate will soon be precipitated in the mixture in the form of crystalline scales of violet colour. Further amounts of the salt may be recovered from the mother-lye.

## Example 3

100 parts of properly bated sheep skins are subjected to a tanning treatment as described in Example 2 with the modification that the alkalinity of the tanning liquor is controlled to 45 amount to 33 per cent from the beginning.

## Example 4

The tanning treatment of the skins is accomplished as described in Example 3, but with the tanning liquor rendered basic as required and divided into several portions which are added at intervals in succession.

## Example 5

100 parts of bated calf skins are fulled in 500

parts of a 4 per cent solution of naphthalino-sulfonic acid for one hour and subsequently 15 to 20 parts of chrome alum are added to the solution. The alkalinity of the tanning solution is kept first at 20 per cent and later on at 33 per cent.

*Example 6*

10 100 parts of calf skins from which the hair has been removed by steeping in lime or the like, are freed from adhering lime by treating the same with a solution of naphthaline-sulfonic acid, whereupon the thus prepared skins are subjected to a treatment with chrome-naphthalino-sulfonate or with a naphthalino-sulfonic acid 15 and an inorganic chromic salt, for the tanning purpose, the alkalinity of the tanning liquor being kept first at 20 per cent and subsequently at 33 per cent.

20 Obviously the alkalinity can be controlled or adjusted differently and kept at a higher degree at the beginning or at the termination of the treatment just depending upon the quality of the leather desired to be obtained.

25 In case of using chromic salts of substituted aromatic sulfonic acids devoid of tanning capacity such as alkylized naphthalino-sulfonic acids, the process is to be carried out similarly as described in the foregoing examples.

30 What I claim is:—

1. The method of tanning hides and skins for the purpose of producing a chrome leather adapted to be soaked again, which comprises preparing the hides and skins in a suitable manner and tanning the same subsequently by means 35 of chromic salts of aromatic sulfonic acids which in themselves possess no tanning properties.

2. The method of tanning hides and skins for the purpose of producing a chrome leather adapted to be soaked again, which comprises preparing the hides and skins in a suitable preparatory treatment and tanning the same subsequently by means of chromic salts of aromatic sulfonic acids having a plurality of nuclei and which possess no tanning properties in themselves.

3. The method of tanning hides and skins for the purpose of producing a chrome leather adapted to be soaked again, which comprises preparing the hides and skins in a suitable preparatory treatment and tanning the same subsequently by means of chromic salts of substitution products of aromatic sulfonic acids which in themselves possess no tanning capacity.

4. The method of tanning hides and skins for the purpose of producing a chrome leather adapted to be soaked again, by means of a chrome tanning process, wherein chromic salts of aromatic sulfonic acids which in themselves possess no tanning properties, are formed in the leather from the components thereof, whereupon, at the commencement of tanning the free, aromatic sulfonic acids will contain at least one-third of the equi-molecular quantity of the chromic salts.

5. The method of tanning hides and skins for the purpose of producing a chrome leather adapt-

ed to be soaked again, which comprises subjecting the hides and skins to a suitable preparatory treatment, treating the prepared hides and skins first with an aromatic sulfonic acid devoid of tanning properties and subsequently with a chromic salt of such an aromatic sulfonic acid, whereupon, at the commencement of tanning the free, aromatic sulfonic acids will contain at least one-third of the equi-molecular quantity of the chromic salts.

6. The method of tanning hides and skins for the purpose of producing a chrome leather adapted to be soaked again, which comprises subjecting the hides and skins to a suitable preparatory treatment, treating the prepared hides and skins first with an aromatic sulfonic acid devoid of tanning faculties, and subsequently treating the same with a solution containing an aromatic sulfonic acid devoid of tanning faculties and a chromic salt of any other suitable acid, whereupon, at the commencement of tanning the free, aromatic sulfonic acids will contain at least one-third of the equi-molecular quantity of the chromic salts.

7. In the method of tanning hides and skins for the purpose of producing a chrome leather adapted to be soaked again, the step of tanning the hides and skins which have not been previously subjected to a pickling treatment, with chromic salts of aromatic sulfonic acids which latter are in themselves devoid of tanning properties, whereupon, at the commencement of tanning the free, aromatic sulfonic acids will contain at least one-third of the equi-molecular quantity of the chromic salts.

8. The method of tanning hides and skins for the purpose of producing a chrome leather adapted to be soaked again, which comprises subjecting the hides and skins to a suitable preparatory treatment, treating the prepared hides and skins first with an aromatic sulfonic acid devoid of tanning properties and subsequently with a chromic salt of such an aromatic sulfonic acid, whereupon, at the commencement of tanning the free, aromatic sulfonic acids will contain at least one-third of the equi-molecular quantity of the chromic salts, while after the liming none of the usual methods is used which effect the deliming and the decaying of the hide.

9. The method of tanning hides and skins for the purpose of producing a chrome leather adapted to be soaked again, which comprises subjecting the hides and skins to a suitable preparatory treatment, treating the prepared hides and skins first with an aromatic sulfonic acid devoid of tanning faculties, and subsequently treating the same with a solution containing an aromatic sulfonic acid devoid of tanning faculties and a chromic salt of any other suitable acid, whereupon, at the commencement of tanning the free, aromatic sulfonic acids will contain at least one-third of the equi-molecular quantity of the chromic salts, while after the liming none of the usual methods is used which effect the deliming and the decaying of the hide.

MAX BERGMANN.